

## UNITED STATES PATENT OFFICE

2,419,144

## ANTISEIZE AND SEALING COMPOUND

John P. Kelly, Toledo, Ohio, assignor to Champion Spark Plug Company, Toledo, Ohio, a corporation of Delaware

No Drawing. Application December 18, 1944,  
Serial No. 568,788

3 Claims. (Cl. 252—23)

1

This invention relates to a compound for use between close fitting metal surfaces to effect a gas tight sealing of the joint therebetween and which at the same time is of a character to prevent seizing of the contacting surfaces, thereby permitting a comparatively easy relative movement of the surfaces when it is desired to effect a separation thereof after conditions of use which may have a tendency to unite or seize the parts in assembled relation.

The invention is especially intended for use in connection with threaded fittings, and more particularly those subjected in use to high temperatures, such for instance as the threaded joints between spark plug shells and the cylinder heads of internal engines in which mounted.

In the use of aviation engines, considerable difficulty is encountered by reason of the sealing or lubricating compounds, commonly used between the cylinder head and spark plug threads, becoming thinned and thus releasing and flowing from the threads under the high temperature conditions to which subjected. This thinning action not only destroys or lessens the joint sealing characteristics of the compound but permits the contacting metal surfaces to seize and prevent relative movements of the surfaces without injury thereto.

The primary object of the invention is the provision of a new and useful compound of the character described, particularly adapted for use in high temperatures between threaded surfaces to prevent seizing of the surfaces so that a comparatively easy separation or relative moving of the surfaces may be effected without injury thereto, and also being of a character to prevent thinning and flowing of the lubricant or sealing agent from between the surfaces under high temperature conditions.

Other objects and advantages thereof will be apparent from the following detailed description of the invention.

A compound embodying the invention that has given highly efficient results in connection with spark plugs used in connection with the mounting of spark plugs in aviation engines comprises the following ingredients mixed in substantially the proportions noted:

|                                  | Per cent |
|----------------------------------|----------|
| Aviation lubricating oil         | 38       |
| Stearate (lithium or barium)     | 12       |
| Talc (magnesium silicate)        | 21       |
| Graphite (preferably flake)      | 23       |
| Corrosive preventive concentrate | 6        |

2

having the following specifications: gravity, A. P. I., 27.5°; flash point, 495° F. to 500° F.; Saybolt viscosity 97 to 102 seconds at 210° F.; viscosity index, 104. Oils having substantially these constants have been found satisfactory in the present composition.

The corrosive preventive concentrate may be made from the following specifications:

Parts

|                                                                                                                                      |    |
|--------------------------------------------------------------------------------------------------------------------------------------|----|
| 10 (a) Petroleum lubricating oil of Saybolt viscosity 750 seconds at 100° F.                                                         | 85 |
| (b) Oil solution of sodium salts of oil soluble sulphonate acids, formed on treating petroleum oils with concentrated sulphuric acid | 10 |
| (c) Degas (a fatty oil that has been extracted from sheep wool, and neutralized with calcium oxide)                                  | 5  |

20 This ingredient may be omitted in compounds used on surfaces that will not corrode.

The lithium or barium stearate is used in powder form and is preferably of a fineness to pass through a U. S. standard 140 mesh sieve. The lithium stearate which has been used with good results in the composition has a melting point of 215° to 221° C.

The talc or magnesium silicate is used in powder form and is preferably white and of a fineness to pass through a U. S. standard 325 mesh sieve and should be free of gritty matter.

The graphite, which is preferably flaked, should be free of gritty matter and in the finished compound be preferably of a fineness to pass 100% through a U. S. standard 120-170 mesh sieve.

It is found in practice that while the preferred compound is mixed in the proportions above-noted, any of these may be varied within the following limits:

|                                  | Per cent |
|----------------------------------|----------|
| Aviation lubricating oil         | 34-44    |
| Stearate (lithium or barium)     | 9-15     |
| Talc (magnesium silicate)        | 17-25    |
| Graphite                         | 19-27    |
| Corrosive preventive concentrate | 0-10     |

In preparing the mixture in small quantities, the following procedure has been followed: The oil compound and the corrosive preventive concentrate are first mixed together and during slow mixing of these the stearate is added and the mixing continued long enough to completely disperse the stearate in the mix. The slow mixing eliminates "throwing-out" of the stearate. The 55 talc and graphite ingredients are added while

The oil component is preferably a refined oil

the oil, corrosive preventive concentrate and the stearate are being stirred and the stirring should continue until a smooth homogeneous mass is obtained. Thorough mixing is essential. The ingredients should be in a cold or unheated state while mixing.

An important advantage of this compound is that the ingredients will remain in suspension for a much longer time than other compounds for similar purposes, of which I am aware. Further, the compound, due to a jelling action under high temperatures, does not flow as freely as other compounds for the purpose and, therefore, effects a more efficient seal and also has a greater tendency to cling and remain on the threads or other surfaces to which applied.

The oil, stearate, graphite and talc each has a particular lubricating quality, and when these ingredients are combined they have such a co-operative action as to form a highly efficient seal and an anti-seize for threaded connections of metal parts, such for instance as spark plugs in aviation engines, subject to use under high temperature conditions, and wherein it may be desirable to disconnect the parts after use for inspection or replacement.

Having thus described my invention, what I claim as new, and desire to secure by United States Letters Patent, is:

1. A composition of matter for use between metal joint surfaces to prevent seizing of the surfaces after heating and cooling cycles comprising 34 to 44% petroleum lubricating oil, 9 to 15% of a stearate of the group consisting of lithium stearate and barium stearate, 11 to 25% talc, and 19 to 27% flaked graphite.

2. A composition of matter for use between

metal joint surfaces to prevent seizing of the surfaces comprising 34 to 44% petroleum lubricating oil, 9 to 15% lithium stearate, 11 to 25% talc, and 19 to 27% flaked graphite.

3. A composition of matter for use between metal joint surfaces to prevent seizing of the surfaces comprising 34 to 44% aviation lubricating oil, 9 to 15% lithium stearate, 17 to 25% talc, and 19 to 27% flaked graphite thoroughly mixed, the stearate being capable of passing through a substantially 140 mesh sieve, the talc being capable of passing through a substantially 325 mesh sieve and the graphite in the finished compound being capable of passing 100% through a 120-170 mesh sieve.

JOHN P. KELLY.

#### REFERENCES CITED

The following references are of record in the file of this patent:

#### UNITED STATES PATENTS

| Number    | Name       | Date           |
|-----------|------------|----------------|
| 1,982,199 | Brunstrum  | Nov. 27, 1934  |
| 2,173,003 | Place      | Sept. 12, 1939 |
| 2,206,025 | Buffington | July 2, 1940   |
| 2,245,702 | Morway     | June 17, 1941  |
| 278,067   | Williamson | May 22, 1883   |
| 2,102,214 | Parker     | Dec. 14, 1937  |
| 2,262,689 | McDowell   | Nov. 11, 1941  |
| 2,345,198 | Hodson     | Mar. 28, 1944  |
| 2,351,384 | Woods      | June 13, 1944  |

#### OTHER REFERENCES

Klemgard (Lubricating Greases), 1937. (Copy in Div. 64, page 722.)